

## UNITED STATES PATENT OFFICE

2,338,677

NONDIFFUSING SULPHONAMIDE COUPLER  
FOR COLOR PHOTOGRAPHYArnold Weissberger, Rochester, N. Y., assignor to  
Eastman Kodak Company, Rochester, N. Y., a  
corporation of New JerseyNo Drawing. Original application August 22,  
1940, Serial No. 353,669, now Patent No.  
2,298,443, dated October 13, 1942. Divided and  
this application May 1, 1942, Serial No. 441,278.  
In Great Britain April 24, 1940

8 Claims. (Cl. 95—6)

This invention relates to photographic color forming compounds and particularly to non-diffusing coupler compounds containing sulphonamide groups for incorporation in photographic emulsion layers.

This application is a division of Weissberger application Serial No. 353,669, filed August 22, 1940, now Patent No. 2,298,443, issued October 13, 1942.

Color forming compounds which react with the development product of aromatic amino developing agents to form colored images on photographic development have been the subject of numerous prior patents. The dyes formed in this way are insoluble in water and in the ordinary photographic developing and fixing baths, although the silver images formed simultaneously with them during the photographic development may be removed from the photographic layer to leave pure dye images in the layer. Such a compound which is employed in conjunction with the developing agent for the silver and which couples with the development product of the developer during photographic development is referred to herein as a coupling component or coupler. When these coupling components are incorporated in the photographic layer prior to exposure, they do not affect the exposure and development of the layer in the usual way but when the development is carried out with a suitable developing agent they combine with the oxidation product of the developer to form a colored image in situ with the silver image.

In Vittum, Peterson and Porter U. S. application Serial No. 404,235, filed July 26, 1941, a continuation-in-part of U. S. Patent No. 2,271,238, granted January 27, 1942, coupling components are described which contain sulphonamide groups. Such couplers are desirable by reason of their solubility characteristics and the improved properties of the dyes formed from them. The couplers described in the Vittum, Peterson and Porter applications are, in general, soluble in the developing solution and not suitable for use in the emulsion layer because of their tendency to diffuse from the layer. The dyes formed from these couplers, however, have better light transmission characteristics and are more stable to heat and light than the dyes produced from previously known coupling components.

It is an object of the present invention to provide coupling components which have the desirable properties of couplers containing the sulphonamide group, which may be incorporated

in photographic emulsion layers as non-diffusing compounds. A further object is to provide novel photographic couplers having desirable properties with respect to heat and light stability. A still further object is to provide photographic couplers which form image dyes having desirable light transmission characteristics. Other objects will appear from the following description of my invention.

These objects are accomplished by replacing the free hydrogen atom of the sulphonamide group of couplers containing such group with radicals having the property of rendering the couplers non-diffusing in gelatin or other colloidal media.

The color forming or coupler compounds which I have found to be suitable for incorporation in silver halide emulsion layers according to my invention are compounds having the following general structure:



where X is alkyl or phenyl substituted alkyl and Y is any organic substituent such as alkyl or aryl.

30 My invention may be illustrated by reference to the following Compounds I and II.



II

45

50

55

Compound I is a coupler capable of producing a yellow dye image and is of the type described in Vittum, Peterson and Porter U. S. application Serial No. 266,152, now Patent No. 2,271,238, issued January 27, 1942. It is soluble in photographic developing solutions. Compound II is identical with Compound I except that the free

hydrogen atom of the sulphonamide group has been replaced with a methyl radical. Compound II also produces a yellow dye upon development with the proper photographic developing agent. However, because of the replacement of the hydrogen atom of the sulphonated group with a suitable radical, the coupler is no longer soluble in the developer but may be incorporated in a photographic emulsion layer as a non-diffusing compound. My invention resides in the discovery that, by the substitution of this free hydrogen atom of the sulphonamide group with suitable organic radicals, the valuable properties of the sulphonamide couplers may be retained, but the solubility properties of the coupler are materially altered and the coupler is rendered non-diffusing in gelatin or other colloidal media.

Compounds suitable for use as non-diffusing couplers according to my invention are as follows:

- 1.
- 2.
- 3.
- 4.
- 5.
- 6.
- 7.
- 8.
- 9.
- 10.
- 11.
- 12.
- 13.
- 14.
- 15.
- 16.
- 17.

One of the substituents on the nitrogen atom of the sulphonamide group, that is, Y in the general formula above, may be any organic substituent such as an alkyl or an aryl radical. The

other substituent on the nitrogen atom, that is, X in the general formula above, is limited to alkyl, phenyl substituted alkyl or benzyl radicals. This is the substituent which controls the solubility of the coupler and produces the property of non-diffusability in gelatin. This substituent may be a simple methyl or ethyl radical or a phenyl substituted alkyl radical such as benzyl or  $\gamma$ -phenylpropyl. These radicals obviously may be considered phenyl substituted alkyl radicals, benzyl being a phenyl substituted methyl radical and  $\gamma$ -phenylpropyl being a phenyl substituted propyl radical.

These couplers contain a methylene group which is reacted with the oxidation product of primary aromatic amino developing agents to produce a dye image on photographic development. The  $\text{CH}_2$  group is present between two negative centers in the group  $-\text{CO}-\text{CH}_2-\text{CN}$  and is, therefore, reactive with the developing agent to produce a dye. 20

The aromatic amino developing agents used with the coupler compounds of my invention include the mono-, di- and tri-aminoaryl compounds and their derivatives formed by substitution in the amino group as well as in the ring, such as alkylphenylenediamines and alkyl toluylenediamines. These compounds are usually used in the salt form, such as the hydrochloride or the sulphate, which are more stable than the amines themselves. Suitable compounds are diethyl-p-phenylenediamine hydrochloride, mono-methyl - p-phenylenediaminehydrochloride, di-methyl - p-phenylenediaminehydrochloride and dimethyl-p-phenylenediamine sulphate. The p-amino-phenols and their substitution products may also be used where the amino group is unsubstituted. All of these compounds have an unsubstituted amino group which enables the oxidation products of the developer to couple with the color forming compounds to form a dye image. 30

The following examples are illustrative of developing solutions which may be used to develop emulsion layers containing the couplers made according to my invention. 40

#### Example 1

|                                |       |     |
|--------------------------------|-------|-----|
| p-Aminodiethylaniline sulphate | grams | 2.5 |
| Sodium sulphite anhydrous      | do    | 2   |
| Sodium carbonate anhydrous     | do    | 20  |
| Potassium bromide              | do    | 1   |
| Water to                       | liter | 1   |

#### Example 2

|                                     |       |    |
|-------------------------------------|-------|----|
| p-Aminodiethylaniline hydrochloride | grams | 2  |
| Sodium sulphite anhydrous           | do    | 5  |
| Sodium carbonate anhydrous          | do    | 20 |
| Potassium bromide                   | do    | 2  |
| Water to                            | liter | 1  |

The couplers used according to my invention may be incorporated in silver halide emulsion layers in various ways but I prefer to form a solution of the sodium salt of the coupler in alcohol and add this to the emulsion. For example, 3 grams of coupler may be dissolved or suspended in 50 cc. of ethyl alcohol and sodium hydroxide added in the amount of 1½ equivalent weights of the coupler. The sodium hydroxide may be added as solid or as a concentrate solution. The sodium salt of the coupler is thereby generated in a solution of 50 cc. of alcohol and this solution is added to 1 liter of a gelatin silver 70

halide emulsion. The pH of the emulsion may then be adjusted if desired by adding a suitable acid such as acetic or sulphuric acid to neutralize all or part of the sodium hydroxide used to form the sodium salt of the coupler. 5

The coupling components may be incorporated either in gelatin or in other colloidal materials such as collodion, organic esters of cellulose or synthetic resins. The emulsion may be carried by a transparent medium such as glass, cellulose ester, or synthetic resin or a non-transparent reflecting medium such as paper or an opaque cellulose ester. The emulsion may be coated as a single layer on the support or superposed layers containing the couplers may be coated on one or both sides of the support. The superposed layers may be differentially sensitized for the formation of a natural color image in the well known manner. 15

The examples and compounds set forth in the present specification are illustrative only and it is to be understood that my invention is to be taken as limited only by the scope of the appended claims. 25

I claim:

1. A photographic emulsion for forming colored images comprising a colloidal carrier containing a sensitive silver halide and a coupler compound having the formula:



where X is selected from the class consisting of alkyl and phenyl substituted alkyl radicals and Y is selected from the class consisting of alkyl and aryl radicals. 30

2. A photographic emulsion for forming colored images comprising a colloidal carrier containing a sensitive silver halide and a coupler compound having the formula:



where X and Y are alkyl radicals. 45

3. A photographic emulsion for forming colored images comprising a colloidal carrier containing a sensitive silver halide and a coupler compound having the formula:



where X is an alkyl radical and Y is an aryl radical. 55

4. A photographic emulsion for forming colored images comprising a colloidal carrier containing a sensitive silver halide and a coupler compound having the formula:



where X is a phenyl substituted alkyl radical and Y is an aryl radical. 65

5. In the method of producing a colored photographic image in a gelatino silver halide emulsion layer, the step which comprises treating the ex-

posed layer containing a coupler compound having the formula:



where X is selected from the class consisting of alkyl and phenyl substituted alkyl radicals and Y is selected from the class consisting of alkyl and aryl radicals, with a developer containing a primary aromatic amino developing agent.

6. In the method of producing a colored photographic image in a gelatino silver halide emulsion layer, the step which comprises treating the exposed layer containing a coupler compound having the formula:



where X and Y are alkyl radicals, with a developer containing a primary aromatic amino developing agent.

7. In the method of producing a colored photographic image in a gelatino silver halide emul-

sion layer, the step which comprises treating the exposed layer containing a coupler compound having the formula:



10 where X is an alkyl radical and Y is an aryl radical, with a developer containing a primary aromatic amino developing agent.

15 8. In the method of producing a colored photographic image in a gelatino silver halide emulsion layer, the step which comprises treating the exposed layer containing a coupler compound having the formula:



20 where X is a phenyl substituted alkyl radical and Y is an aryl radical, with a developer containing a primary aromatic amino developing agent.

ARNOLD WEISSBERGER.

CERTIFICATE OF CORRECTION.

Patent No. 2,338,677.

January 4, 1944.

ARNOLD WEISSBERGER.

It is hereby certified that error appears in the printed specification of the above numbered patent requiring correction as follows: Page 2, second column, lines 62 and 68, Formulas 15 and 16 respectively, for that portion reading " $\text{CH}_2\text{-CH}$ " read -- $\text{CH}_2\text{-CN--}$ ; and that the said Letters Patent should be read with this correction therein that the same may conform to the record of the case in the Patent Office.

Signed and sealed this 3rd day of October, A. D. 1944.

Leslie Frazer

(Seal)

Acting Commissioner of Patents.